

## UNITED STATES PATENT OFFICE

2,071,481

## DYED LUBRICATING OIL

Carl Winning and Stewart C. Fulton, Elizabeth,  
N. J., assignors to Standard Oil Development  
Company, a corporation of Delaware

No Drawing. Application November 16, 1931,  
Serial No. 575,461

1 Claim. (Cl. 196—151)

This invention relates to a dyed lubricating oil. The dye is obtained from tars produced in the cracking of petroleum products, but these are not used as such as additions to oils, in our product. The invention will be fully understood from the following description.

In the co-pending application Ser. No. 572,059 filed October 30, 1931 by Stewart C. Fulton a process has been described for obtaining resins from heavy petroleum products, especially cracked tars of petroleum origin. Briefly this process consists of removing most of the oily constituents from the cracked tar by distillation preferably under vacuum and agitating or digesting the residual product with a light petroleum hydrocarbon solvent, such as naphtha, to dissolve the resins therefrom and to obtain asphaltenes as residual product. The naphtha solution is then acid treated, neutralized either with finely divided clay or by washing, and distilled to remove the solvent. The residual product is a resin having the following properties:

|                                           |                                |
|-------------------------------------------|--------------------------------|
| Softening point<br>(ball and ring method) | Above 80° F.                   |
| Color                                     | Reddish brown                  |
| Streak on porcelain                       | Yellow to reddish brown        |
| Odor                                      | None                           |
| Taste                                     | None                           |
| Solubility                                | (Light naphtha, gasoline, etc. |
|                                           | Linseed oil                    |
| Solubility                                | China wood oil                 |
|                                           | Esters, such as amyl acetate   |
| Insoluble in                              | Benzol                         |
|                                           | Water                          |
| Insoluble in                              | Lower alcohols                 |
|                                           | Acetone                        |

We have discovered that resins obtained from cracked tars of petroleum origin by separating the oily products and asphaltenes from the resin, are good materials for dyeing lubricating oils. Such resins may be prepared by the above described method, or by other methods also. The resin may be added either to a lubricating oil distillate or to a cylinder oil when a darker color is desired, or it may be added to the so-called pale oils to give them a desired shade of color. In all cases the cast of the oil dyed by the addition of such resins is greatly improved inasmuch as these resins impart a desirable olive green cast to the oils dyed therewith.

The resin may be dissolved in a lubricating oil by agitation, with slight warming in case of a viscous oil. It is preferable to prepare first an intermediate solution by dissolving say 10% by weight of resin in a certain portion of the oil and use this intermediate solution for dyeing large quantities. The amount of resin in the final dyed lubricating oil product is usually less than

about 1%. Solutions of the resin in other solvents may of course be used. For example, a concentrate of the resin in the solvent employed in the resin-separating process, such as kerosene, may be added to the lubricating oil. The amount of solvent required to be used is too small to affect the properties of the oil.

The following example will illustrate our process and the products obtained. A pale lubricating oil prepared by vacuum pipe still operation from Colombia crude was divided into two lots and dyed with a resin obtained from cracking coil tar by first preparing an intermediate solution and then adding varying amounts of this intermediate solution to the two lots of lubricating oil. The following table will show the inspection of the original product and the dyed products:

|                                                                                       | Original oil | Dyed oil No. 1 | Dyed oil No. 2 | 20 |
|---------------------------------------------------------------------------------------|--------------|----------------|----------------|----|
| Oil dye, % by weight                                                                  | 0.0          | 0.2            | 0.7            |    |
| Gravity, A. P. I.                                                                     | 23.1         | 23.0           | 22.9           |    |
| Flash °F.                                                                             | 420          | 420            | 420            |    |
| Viscosity @ 100° F. (Saybolt)                                                         | 520          | 524            | 535            |    |
| Viscosity @ 210° F. (Saybolt)                                                         | 57.4         | 57.4           | 57.6           | 25 |
| Viscosity index                                                                       | 54           | 55             | 51             |    |
| Color (Robinsson)                                                                     | 104          | 4½             | 13/            |    |
| Pour °F.                                                                              | —5           | —5             | —10            |    |
| Color after heating 16 hrs. @ 210° F.                                                 | 1/4          | 1/2            | 1/4            |    |
| S. E. (steam emulsion number as defined in A. S. T. M. report of Committee D-2, 1932) | 170          | 195            | 231            | 30 |
| Conradson carbon, %                                                                   | 0.02         | 0.08           | 0.22           |    |
| Cast                                                                                  | Poor         | Good           | Good           |    |

The present invention permits of imparting the desired cast or fluorescence to the lubricating oil and to effect other improvements. Thus we have observed that the pour point of certain lubricating oils, such as for example the pour of light and medium hydrogenated oils, is lowered by the incorporation of resins prepared from cracked tars of petroleum origin.

Our invention may be used with special advantage to the preparation of lubrication oils known in the trade under the name of "red oils". A great many users of lubricating oils demand red oils in preference to the lighter colored pale oils. Many red oils on the market are blends of pale oils with sufficient viscous red oil (bright stock) to yield the desired color. The sought for color of red oils can be obtained by the addition of our dye concentrate which does not cause the impairment in oil quality attendant to the use of bright stock blends. The following example gives the inspection of a pale oil and of two red oils prepared from the pale oil, one by

5

10

15

35

40

45

50

55

the addition of 5% bright stock and the other one by the addition of 0.08% resin:

|                              | Pale oil | Pale oil+5% bright stock | Pale oil+0.08% resin |
|------------------------------|----------|--------------------------|----------------------|
| 5 Gravity A. P. I.           | 27.1     | 26.9                     | 27.1                 |
| Viscosity Saybolt at 210° F. | 53.2     | 54                       | 53.4                 |
| Color Tag.—Robinson          | 14       | 9                        | 9                    |
| Carbon residue               |          | 0.07                     | 0.01                 |
| 10 Pour ° F.                 | 0        | 0                        | -15                  |

It is seen that the red oil prepared with the resin is of a superior quality in comparison to the red oil of the same color prepared by the addition of bright stock as proved by the Conradson carbon test. The pour of the red oil prepared with the resin was also lower than that of the original pale oil or that of the red oil prepared by the addition of bright stock. The steam emulsion number is also better when the red oil is prepared with resin.

The amount of resin to be added to the pale

oil depends on the desired color of the red oil. Usually this amount is below 1% but in some cases it may be higher, 2-5% or even higher.

Our invention is not to be limited by the particulars given by way of illustration but merely by the following claim in which it is our intention to claim all novelty inherent in the invention.

We claim:

A lubricating oil containing a pour point depressant and bloom agent prepared by distilling cracked petroleum residue to remove the oily constituents therefrom, extracting the distilled residue with a solvent in which asphaltenes are substantially insoluble, subjecting the extract containing the solvent to acid treatment, neutralizing the acid treated solvent extract and distilling off the solvent to form the pour point depressant and bloom agent.

CARL WINNING.  
STEWART C. FULTON.

20

15